

E. H. MEYER & J. M. A. STILLESEN.  
ELECTROCHEMICAL APPARATUS AND PROCESS.  
APPLICATION FILED MAR. 20, 1908.

965,393.

Patented July 26, 1910.

2 SHEETS—SHEET 1.



Fig. 1

Witnesses  
A. K. Schneider  
Edmund O. Duborg.

Inventors  
E. H. Meyer &  
J. M. A. Stillesen,  
By their Attorneys  
Edward, Lager & Wooster.

E. H. MEYER & J. M. A. STILLESEN.  
ELECTROCHEMICAL APPARATUS AND PROCESS.  
APPLICATION FILED MAR. 20, 1908.

965,393.

Patented July 26, 1910.

2 SHEETS—SHEET 2.



Fig. 2

Witnesses  
A. K. Schneider  
Edmund C. Duboy.

E. H. Meyer & Inventors  
By their Attorneys J. M. A. Stilleesen  
Edwards, Lager & Wooster.

# UNITED STATES PATENT OFFICE.

EINAR HONORATUS MEYER AND JOB MORTEN AUGUST STILLESEN, OF NIAGARA FALLS, ONTARIO, CANADA.

## ELECTROCHEMICAL APPARATUS AND PROCESS.

965,393.

Specification of Letters Patent. Patented July 26, 1910.

Application filed March 20, 1908. Serial No. 422,240.

To all whom it may concern:

Be it known that we, EINAR HONORATUS MEYER and JOB MORTEN AUGUST STILLESEN, subjects of the King of Norway, residing at 5 Niagara Falls, in the Dominion of Canada, have invented certain new and useful Improvements in Electrochemical Apparatus and Processes, of which the following is a full, clear, and exact specification.

10 This invention relates to electro-chemistry, and has particular reference to a process of, and apparatus for, producing calcium carbide continuously from the raw materials, limestone and coal, without loss of heat or of 15 by-products.

In the treatment of lime and carbon in the electric furnace to form calcium carbide, carbon monoxide is produced, while to reduce the limestone to lime, and coal to carbon, heat is required, which heat, according to this invention, is produced by the combustion of the carbon monoxide from the carbide furnace with air. The gaseous products from the limestone and coal retort consist principally of carbon dioxide and nitrogen, and the invention further comprises a process and apparatus whereby the nitrogen can be isolated and combined with calcium carbide to form calcium cyanamide.

30 The invention with reference to the apparatus, will be more fully understood in connection with the description of the accompanying drawings, and the process will be understood in connection with the description of the operation of the apparatus.

In the drawings, Figure 1 is an elevation, partly in section, of the apparatus. Fig. 2 is a diagrammatic view showing the connections between the parts of the apparatus. 40 1 is a stack built of a common brick and supported in the manner shown. The upper half 2, built of refractory material, forms a retort for the reduction of limestone into lime and coal into carbon. Both the limestone and coal are fed in through the feeding apparatus 4 in a finely crushed form. After the limestone has been reduced to lime and the coal to carbon, the charge is dropped down into the receiver 3 (built of 45 refractory material), from which it is fed down to the furnace 5 by means of pump 6.

The carbide furnace 5 is inclined to the vertical as shown, for the purpose of securing better efficiency, and to enable the charge

to be supplied at the bottom of the furnace 55 at the hottest part.

8 is a movable electrode, and 9 a fixed bowl-shaped electrode, with circuit connections with a source of electricity, not shown.

10 is a motor geared to move the electrode 60 8 toward and from the electrode 9, and controlled in any desired manner.

From the furnace 5 a gas vent pipe 12 connects with rings 13, from which the gas is supplied to the conical burner 14 in the 65 retort 2, after being mixed with air, and burned therein to reduce the coal and limestone. As herein shown, there are three furnaces 5, all supplied from the reservoir 3, and furnishing gas to the burner 14. This 70 burner preferably is conical as shown, and consists of pipes having perforations at the bottom, so that they will not become clogged by the charge. Acetylene or other gas can be supplied to a pilot burner 15 to insure 75 ignition of the monoxide at the burner and the gases from the coal. These burners are located under a finely meshed grate 16.

In Fig. 2 is shown a diagram of the piping for the burners and the controlling 80 valves, a number of which are used for independently controlling sections of the burners, so that the heat can be minutely controlled. A sufficient supply of air is admitted with the gas to burn all the gases in 85 the retort 2 to carbon dioxide and water, so that the gases passing out at the top through pipe 18 will consist principally of carbon dioxide and nitrogen. A valve controls the admission of air. Pipe 18 leads 90 through a cooler (not shown), thence to a tank 19 containing calcium hydrate, which absorbs the water and carbon dioxide, but not the nitrogen which was introduced as a part of the air. From tank 19 the nitrogen 95 passes by pipe 20 through a fan 22, to a drier, not shown, thence through a pipe 23 to the cyanamide furnace 25. This latter furnace consists of an air-tight drum on a foundation 26, and is heated by carbon monoxide gas from the carbide furnace, if desired, ignited by acetylene or other means.

In carrying out the process of the invention, whereby calcium carbide is made from the raw material, the coal and limestone charged into retort 2 is admitted to reservoir 3 and thence fed while still hot into the furnace 5, and thence the melted carbide

when formed, is tapped out from the bottom of the furnace 5, and is ready for use after being cooled and crushed, in making calcium cyanamid, or for other purposes.

5 The carbid made by the continuous process for raw material newly burned and yet warm, does not cool the furnace upon its introduction, and is furthermore fed in at the bottom, at the hottest portion, so that

10 carbid is produced at a small outlay of electric energy.

The process of extracting nitrogen consists in passing the gases from the retort (sufficient air having been admitted with

15 the gas to consume all the monoxid and hydrocarbons), and then passed through the calcium hydroxid.

So far as we are aware, it has not heretofore been proposed to produce calcium carbid from the raw materials in a single process, nor has it heretofore been proposed to utilize the gaseous products from the reduction of coal and limestone to obtain nitrogen.

25 Having thus described our invention, we declare that what we claim as new and desire to secure by Letters Patent, is:—

1. The process of making calcium carbid comprising reducing a mixture containing

30 coal and limestone to carbon and lime in a separate chamber by the combustion of a gas containing carbon monoxid in intimate contact with said mixture, feeding the reduced carbon and lime without cooling from

35 said chamber into an electric furnace, and subjecting the same therein to the action of an electric arc.

2. The process of making calcium carbid comprising treating a mixture comprising

40 lime and carbon in an electric arc, burning the resultant evolved carbon monoxid with addition of air in direct contact with limestone and coal contained in a separate chamber to produce lime and carbon, and dis-

45 charging the lime and carbon from said chamber without cooling into an electric arc.

3. The process of making calcium carbid comprising forming an arc between a plurality of electrodes feeding reduced lime

50 and carbon directly into said arc, conducting liberated carbon monoxid with addition of air into a mass of coal and limestone contained in a separate reducing chamber and igniting the same to reduce said mass to a

55 mixture of carbon and lime, and discharging the freshly formed carbon and lime downwardly from said reducing chamber into a reservoir from which the same may be fed into an electric arc while still hot.

60 4. The process of making calcium carbid comprising reducing a mixture of coal and limestone to carbon and lime by leading into said mixture a combustible gas containing carbon monoxid and burning the same

65 therein, collecting the reduced mixture of

carbon and lime in a separate inclosure as a mass and withdrawing from said collected mass a desired quantity without cooling, charging the same into an electric furnace and subjecting the same therein to the action of an electric-arc.

5. The process of making calcium, carbid comprising collecting the gas evolved upon subjecting a mixture of carbon and lime to the action of an electric arc, burning said

70 gas together with air in a mixture of coal and limestone to reduce the same to a mixture of carbon and lime; collecting the reduced mixture of carbon and lime as a mass in a separate inclosure, tapping from said

75 inclosure without cooling a desired quantity, and subjecting the same to the action of an electric arc.

6. The process of making calcium carbid comprising collecting the gas evolved upon

80 subjecting a mixture of lime and carbon to the action of an electric arc, adding air to said evolved gas and igniting the resulting mixture of gases in a mixture of limestone and coal contained in a separate reducing

85 chamber, to produce a reduced mixture of lime and carbon, discharging the reduced mixture from said chamber without cooling to a separate chamber, thereby collecting

90 a mass of said reduced mixture in a separate chamber, and tapping from said mass of reduced mixture without cooling any desired quantity and subjecting the same to the action of an electric arc.

7. The process of making calcium carbid

100 comprising collecting the gases evolved upon subjecting a mixture of lime and carbon to the action of an electric arc, leading said evolved gases through a plurality of pipes disposed in the bottom of a retort and opening at said bottom into said retort, igniting said gases in a mixture of coal and limestone supported on said bottom, thereby producing a reduced mixture of carbon and lime, discharging said mixture of carbon

105 and lime into a furnace and subjecting the same to the action of an electric arc.

8. The combination with a carbid furnace, of a retort adapted to contain coal and limestone, means for burning the gases from the furnace in intimate relation with the contents of the retort, whereby to reduce the same to carbon and lime, and means for separating nitrogen from the gases from the

110 retort.

9. The combination with a carbid furnace, of a retort adapted to contain coal and limestone, means for burning the gases from the furnace in intimate relation with the contents of the retort, whereby to reduce the same to carbon and lime, means for separating nitrogen from the gases from the retort, and means for producing calcium cyanamid from the nitrogen so obtained.

10. The process of obtaining nitrogen,

- which comprises conducting the gases evolved from the treatment of a carbid producing charge in an electric furnace, igniting said evolved gases with air, and removing from the gaseous product of such ignition all but nitrogen. 5
11. The process of obtaining nitrogen in electrolytic calcium carbid manufacture, consisting in igniting the gases from the electrolytic furnace with air to reduce coal and limestone, and separating nitrogen from the gaseous products of such combustion. 10
12. The process of obtaining nitrogen consisting in passing a mixture of air and combustible gas through a mass of coal and limestone and igniting the same, and treating the resultant gases with a solution of calcium hydrate whereby to absorb all but nitrogen and water vapor. 15
- 20 13. The process of obtaining nitrogen as a by-product in electrolytic calcium carbid manufacture, consisting in igniting the gases from the electrolytic furnace with air, and then passing the products of such combustion through calcium hydrate. 25
14. A process for obtaining lime, carbon and nitrogen simultaneously, consisting in igniting a mixture of combustible gas and air in intimate relation with coal and limestone to produce carbon and lime, and passing the gaseous products of such combustion through an absorbent of carbon dioxide. 30
- 35 15. A process for obtaining lime, carbon and nitrogen simultaneously with calcium carbid, consisting in forming calcium carbid in an electric arc, igniting the gases therefrom mixed with air in intimate relation with coal and limestone to form carbon and lime, and passing the products of such ignition through an absorbent of carbon dioxide. 40
- 45 16. The process of obtaining nitrogen as a by-product in electrolytic calcium carbid manufacture, consisting in igniting the gases from the electrolytic furnace with air, and then passing the products of such combustion through an absorbent of carbon dioxide. 50
17. The process of obtaining nitrogen consisting in igniting a mixture of carbon monoxide and a predetermined portion of air in intimate relation with limestone to produce lime, and passing the gaseous products of such combustion through an absorbent of carbon dioxide. 55
- 60 18. The process consisting in passing a mixture of air and combustible gas from a carbid furnace through coal and limestone, igniting the same to reduce the coal and limestone, and removing all but nitrogen from the resultant gases. 65
19. The process consisting in collecting the gases evolved from the treatment of a carbid producing charge in a furnace, mixing said gases with air and igniting the same, and passing the resultant gases through calcium hydrate. 70
20. The process of obtaining nitrogen consisting in igniting a mixture of gases evolved from a carbid producing charge and air in intimate relation with limestone to produce lime for another carbid charge, and eliminating carbon dioxide from the gaseous product of such ignition. 75
21. The process of obtaining nitrogen consisting in igniting a mixture of gases evolved from a carbid producing charge and air in intimate relation with limestone to produce lime for another carbid charge, and passing the gaseous products of such ignition through an absorbent of carbon dioxide. 80
22. The process of obtaining nitrogen consisting in igniting a mixture of gases evolved from a carbid producing charge and air in intimate relation with limestone to produce lime for another carbid charge, and removing from the gaseous product of such ignition all but nitrogen. 85
23. The process of obtaining nitrogen consisting in igniting a mixture of gases from an electrolytic furnace and air in intimate relation with limestone to produce lime for another carbid charge, and eliminating carbon dioxide from the gaseous product of such ignition. 90

In testimony whereof we affix our signatures, in presence of two witnesses.

EINAR HONORATUS MEYER.

JOB MORTEN AUGUST STILLESEN.

Witnesses:

HARRY MARSLY,  
AUGUSTUS LOTZAR.